

## UNITED STATES PATENT OFFICE

1,996,314

## FIBROUS COMPOSITION

Gordon E. Wightman, Upper Montclair, N. J.

No Drawing. Original application December 18, 1928, Serial No. 326,911. Divided and this application March 26, 1931, Serial No. 524,207. In Canada December 5, 1929

1 Claim. (Cl. 154—2.8)

This invention relates to fibrous compositions including a bonding agent, and more specifically relates to such compositions supplied in sheet form and intended for the manufacture of laminated products for insulating and kindred purposes. Bonding agents in prevalent use for such compositions are the resinoids, or compounds of a resinous character which can be changed from a fusible, soluble and potentially reactive state to a substantially infusible and insoluble state by the application of heat, since compositions including such bonding agents impart superior electrical and mechanical properties to articles made therefrom. The bonding agents are customarily applied to sheets of the fibrous material as solutions to form coatings or impregnations, and laminated products are made therefrom by superposing a number of coated sheets and simultaneously applying heat and pressure to convert the resinoid binder to the insoluble, infusible condition; but they can be otherwise incorporated with the fibers, for example by the wet process as described in a patent to Baekeland 1,160,362 granted November 16, 1915.

As fibrous material for such compositions, wood pulp is commercially in demand on account of its low cost; but, as heretofore supplied, it has not been found desirable, particularly in compositions of sheet form for laminated products for electrical insulation, on account of the excessive rate of water absorption and/or other properties being such as to render the laminated products formed therefrom less unsatisfactory for this and other purposes, particularly those requiring highest quality.

Contrary to this past experience with wood pulp, I have discovered the compositions can be made from wood fibers, yielding products having a rate of water absorption so low as to compare favorably in this respect with other fibrous insulating materials, such as cotton, and to be otherwise made more suitable for electrical insulation, provided the wood pulp be treated so as to be relatively high in resistant cellulose fibers, that is, provided approximately 90 and preferably 94 per cent or more of the pulp content is alpha cellulose. Such a pulp can be prepared for example by treating or cooking a sulfite pulp, obtained by digesting wood chips in an acid sulfite solution, with an alkaline liquor, such as caustic soda, best followed by bleaching with chlorine or other suitable agent; other methods or modifications thereof known to the paper making art can be employed.

The wood pulp rich in alpha cellulose so ob-

tained can be handled in the same manner as any other fibrous material, and laid into paper or sheet form on a paper making machine after beating to effect a partial hydration of the fibers. Following the usual procedure, the sheet after drying is coated or impregnated with a potentially reactive resinoid in solution and the solvent removed. Any of the known resinoids, for example the phenol-formaldehyde condensation products, or compositions described in a Patent 1,677,417 to Turkington granted July 17, 1928 comprising phenol-fatty-oil methylene reaction products, can be used for this purpose. The resinoids of the Turkington disclosure are tough and elastic when cold and form flexible laminated products with sheets of high alpha cellulose content, from which insulating parts can be stamped out.

A typical sample of laminated material stock, prepared from superposed sheets of paper with an alpha cellulose fiber content of 94 per cent or more bonded with a coating or impregnating composition consisting of a solution of a resinoid made from cresol and formaldehyde and added in amount so as to yield a stock with about 40 per cent resinoid content, and molded under heat at a temperature of about 170° C. and pressure at about 1000 pounds per square inch to convert the resinoid to the substantially infusible state, had a water absorption over a period of 24 hours of about 1.3 per cent; a kraft wood fiber paper stock as used heretofore and similarly prepared showed an absorption of 3.5 per cent. In addition it may be here noted that alpha cellulose pulp is more readily prepared in paper form than kraft pulp and the beating time required for kraft is from one-third to two-thirds longer than that required for alpha-cellulose. In comparative tests with cotton fiber stock, alpha cellulose stock had a higher dielectric strength, 920 volts per mil for alpha cellulose as compared with 840 volts per mil for cotton, and a lower power factor, the alpha cellulose laminated measurement being 1.88 at audio frequency while the cotton fiber stock measured about 3.5. In mechanical properties of tensile and transverse strength and elasticity, cotton, alpha cellulose and kraft laminated pieces tested were of about the same order, alpha cellulose having a somewhat superior tensile strength to the others, or a strength of over 17,000 pounds to the square inch, and less brittleness than the kraft, its modulus of elasticity as measured being about 1,190,000.

5

10

15

20

25

30

35

40

45

50

55

This is a division of my application Ser. No. 326,911, filed Dec. 18, 1928.

I claim:

Laminated stock suitable for electrical insulation comprising superposed sheets of porous wood fibers having an alpha cellulose of at least 90 to 94% bonded with a resinoid and characterized by a dielectric strength greater than 850 volts per mil, power factor less than 3.4, tensile strength greater than 17,000 pounds per square inch and water absorption less than 3 per cent in 24 hours.

ized by a dielectric strength greater than 850 volts per mil, power factor less than 3.4, tensile strength greater than 17,000 pounds per square inch and water absorption less than 3 per cent in 24 hours.

GORDON E. WIGHTMAN.